

Nov. 18, 1941.

D. B. WHEELER ET AL

2,263,200

BACKING SHEET FOR BUILDING INSULATING MATERIALS

Filed May 24, 1938

2 Sheets-Sheet 1



Inventors

DONALD B. WHEELER  
JAMES D. GRIFFIN

By *Norman + Haleman*,  
Attorneys

Nov. 18, 1941.

D. B. WHEELER ET AL

2,263,200

BACKING SHEET FOR BUILDING INSULATING MATERIALS

Filed May 24, 1938

2 Sheets-Sheet 2

*Figs. 6.*



*Figs. 8.*



*Figs. 10.*



*Figs. 11.*



*Figs. 7.*



DONALD B. WHEELER  
JAMES D. GRIFFIN

Morris & Otteman,

Attorneys

## UNITED STATES PATENT OFFICE

2,263,200

BACKING SHEET FOR BUILDING  
INSULATING MATERIALS

Donald B. Wheeler, Hudson Falls, and James D. Griffin, Harrison, N. Y., assignors to Union Bag & Paper Corporation, Hudson Falls, N. Y., a corporation of New Jersey

Application May 24, 1938, Serial No. 209,830

7 Claims. (Cl. 91—70)

The primary object of the present invention is to provide a sheet of paper or similar material having a coating applied thereto which is substantially non-tacky at any ordinary atmospheric temperature but which is capable of being rendered adhesive when heated to an appropriate temperature, and after cooling will effectively maintain its adhesive properties through all ranges of atmospheric temperatures.

It is a more particular object to provide a sheet of this character having a coating applied thereto which is of such a composition that it will not crack or lose its adhesive properties within the limits of temperature from sub-zero to summer heat and which, when applied to the sheet will permit winding of the sheet into a roll without transfer of the composition from the face of the sheet to the back of the adjacent convolutions thereof.

Another object is to provide a flexible sheet of paper or the like having a waterproof composition applied to one side thereof and which is capable of being rendered adhesive by the application of heat thereto, such composition being ribbed to facilitate application of the sheet to other objects or surfaces for adhesive attachment thereto, the marginal edges of the sheet being free of the composition, or substantially so, to render them readily foldable relatively to the body of the sheet, the back of the sheet being preferably also treated to further increase its moisture proof qualities.

Another object of the invention is to provide a novel process of producing a sheet having the foregoing characteristics, it being a further development of the process disclosed in U. S. Patent No. 1,667,691 granted April 24, 1928.

A sheet prepared in accordance with the present invention may be used for various purposes, but it is especially adapted to be applied as a facing and support for the heat insulating material used in the building of houses and other structures, it being capable of application adhesively to the insulating material by applying heat at a suitable temperature, the composition applied to the sheet providing protection to the insulating material against saturation with moisture from wet plaster when applied to the wall and preventing the passage of air, thereby improving the effectiveness of the insulating material, and the sheet serving as a means for holding the insulating material in place, the edges of the sheet extending beyond the insulating material so that they may be applied and secured to studing or other wall supports.

The invention is set forth more particularly with reference to the accompanying drawings wherein:

Figure 1 is a side elevation of an apparatus suitable for use in providing a sheet according to the present invention;

Figure 2 is a detail view of the doctor blade which forms ribs in the composition applied to the sheet;

Figure 3 is a side view of the doctor blade;

Figure 4 is a face view of a portion of a strip having the composition applied thereto;

Figure 5 is a cross section of the strip taken on the line 5—5 in Fig. 4;

Figure 6 is a face view of the strip showing the manner of slitting it longitudinally to form a plurality of strips and of turning the edges of these strips inwardly;

Figure 7 is a section taken diametrically through a roll of the material;

Figure 8 is a perspective view of a completed sheet made in accordance with the present invention;

Figure 9 is a side elevation of an apparatus suitable for use in applying the strip adhesively to a strip of insulating material;

Figure 10 is a perspective view showing a batt of insulating material having the sheet applied adhesively thereto; and

Figure 11 is a perspective view showing the manner of installing and securing the batt in place in a wall.

Similar parts are designated by the same reference characters in the different figures.

In carrying out the present invention according to the preferred process, the continuous strip A of base material, which may be any cellulosic paper but is preferably kraft paper, is supplied from a roll 10 to a heating drum 11, which may be heated by steam or other suitable heating means and which pre-heats the sheet, and the sheet is then directed by guide rollers 12 and 13 to a coating roll 14, the sheet passing over the upper side of this roll the lower side of which is immersed in a bath of the treating composition which is contained in a treating tank 15 and fills the same to the level indicated at X.

The composition contained in the tank 15 and which is applied to the entire lower surface of the travelling strip by the roll 14, is one which will be liquid when heated to a temperature ranging between 300° and 360° F. and when cooled to any ordinary atmospheric temperature will solidify and be substantially non-tacky and waterproof, and when heated after being applied

will possess good adhesive properties. It preferably consists of a bituminous composition composed of a mixture of montan pitch and an asphalt or a pitch. The composition is composed preferably of the following mixture:

50% montan pitch, in its unrefined or raw state.  
50% asphalt, 14 penetration petroleum base,  
having a melting point of 290° to 300° F.

Montan pitch is the residue remaining after the refinement of montan wax by distillation with superheated steam in vacuo. The montan pitch preferably employed is the Riebeck brand imported from Germany, which is of the following analysis:

|                                    |                     |
|------------------------------------|---------------------|
| Melting point according to Kramer- |                     |
| Sarnow method                      | °F. 144 to 153      |
| Acid value                         | 2 to 5              |
| Ester value                        | 3 to 5              |
| Saponification value               | 5 to 10             |
| Insolubles in benzol               | per cent 0.2 to 0.3 |
| Ash                                | do 0.1 to 1.0       |

The asphalt preferably employed and which is available on the market according to specifications is a petroleum base asphalt which is preferably air-blown so that it is free from water or decomposition products, has a specific gravity at 77° F. of not less than 1.003 and a melting point (ball and ring method) not lower than 275° F. and not higher than 300° F. and a flash point, when determined by the Cleveland open cup method, not lower than 500° F. and is soluble in C. P. carbon bisulphide or cold carbon tetrachloride to the extent of at least 99.5% and soluble in 86 degrees Bé. Pennsylvania paraffine naphtha to the extent of not less than 56.0% and not more than 66.0%. Its penetration (Dow method) using a No. 2 needle is as follows:

At 32° F. 60 sec. 200 grams weight, not less than 5;  
At 77° F. 5 sec. 100 grams weight, not less than 7  
nor more than 13;  
At 115° F. 5 sec. 50 grams weight, not more than 18.

Fifty grams of the material upon being maintained at a uniform temperature of 325° F. for five hours in a cylindrical vessel 2½ inches in diameter and 1½ inches high should not lose more than 0.4% by weight.

In place of the asphalt, stearine pitch may be employed in the composition, in the same proportion with the montan pitch as stated above. Such stearine pitch may be mixed with preferably 50% to 60% cotton seed pitch, and is air blown so that it will be free of water and decomposition products and have a melting point of from 190° F. to 200° F. (ball and ring method.)

The composition contained in the tank 15 is maintained in a liquid state by heating it to a temperature ranging between 300° and 360° F., depending upon the texture of the paper and the composition used, which must be kept sufficiently fluid to produce an even coating on the paper without undue penetration of the composition into the paper, a temperature of about 320° F. being preferable when the composition is applied to kraft paper. Any suitable means may be provided for thus heating the composition in the tank 15, electric air heating units 16 being shown for example.

The strip of paper having its entire lower surface coated with the composition by the coating roll 14, passes from said roll over a doctor blade 17 the upper edge of which is adapted to form

the composition on the strip into ribs and to provide substantially uncoated longitudinal areas on the strip. In the present instance, the strip passing through the apparatus is intended to be slitted longitudinally to form two sheets, and the doctor blade is accordingly formed on its upper edge with two sets of ribs 18 and 19, one set for each sheet to be produced, these ribs being preferably inclined in opposite directions, as shown in Fig. 2, so that as the strip passes over the doctor blade, the sets of ribs a and a' in the composition on the strip, the areas of the paper strip intervening the ribs being preferably scraped clear of the composition, or substantially so, and the middle and end portions 20 and 20' respectively of the doctor blade lying in the same plane with the tops of the ribs 18 and 19 so that these portions of the doctor blade will scrape the middle and marginal portions a<sup>2</sup> and a<sup>3</sup> and a<sup>4</sup> respectively clear, or substantially so, of the composition. By inclining the sets of ribs 18 and 19 in reverse directions, they will act to stretch the strip laterally toward its side edges and thus maintain it under tension transversely as it advances, thereby avoiding the formation of pleats in the strip or deflection of the sheet in either direction laterally.

After passing over the doctor blade 17, the sheet having the hot composition on one side thereof, is immediately cooled and thereby hardened or set sufficiently to prevent undue penetration of the composition into the sheet, by passing the sheet around a cooling drum 21, and the sheet is then coated on its other side with a suitable waterproof wax to further increase its vapor and waterproof properties. This is accomplished by passing the sheet over a wax applying roll 22 which is mounted in the upper part of a wax tank 23 containing a wax, preferably paraffine, which is maintained in a liquid state by heating it to a temperature of from about 128° to 130° F. by suitable means such for example as a steam coil 24, the roll 22 dipping into the molten wax, and the surplus wax is removed from the sheet by a doctor blade 25 which scrapes the waxed surface evenly so as to leave an even coating of the wax on the sheet.

The sheet, immediately after the wax coating has been applied thereto, is cooled to harden or set the wax on one side as well as the composition on its other side by passing around a cooling drum 26, and it then passes beneath a slitter 27 which slits the strip longitudinally to form it, for example, into two strips divided by the median longitudinal dotted line in Fig. 4, and these strips then pass over formers 28 which, as shown in Fig. 6, are each of a width corresponding approximately to the width of the ribbed composition thereon, the upper ends of these formers being curved and the formers inclined, as shown in Fig. 1, so that the longitudinal edges of each subdivided strip, as it passes onto its former, will fold downwardly and inwardly toward the lower or waxed side thereof.

Each of the subdivided strips with its longitudinal edges as thus turned and folded, is wound into a roll A' by any suitable means such for example as a pair of winding drums 29 and 30 which may be driven in any suitable manner and serve to support and drive the respective roll by its edges, as shown in Fig. 7, the folded or doubled edges of the sheets which form the rolls providing hard ends on the rolls to rest on the winding drums and thereby protecting the in-

termediate portions of the roll containing the composition from pressure from these drums.

Paper or other flexible material treated according to the present invention is highly flexible and the adhesive composition applied thereto is substantially non-tacky at all ordinary atmospheric temperatures but is rendered highly adhesive when heated to a suitably higher temperature, such as a temperature ranging between 175° and 275° F. and it will not crack or lose its adhesive properties within the limits of from sub-zero temperature to summer heat.

The non-tacky property of the adhesive composition at all ordinary atmospheric temperatures, due to the proportion of the waxy montan pitch constituent of the composition, facilitates the handling of the strip and enables it to be wound into rolls in convenient form for storage or shipment, transfer of the composition on the strip from the face of one convolution to the back of another being further prevented by the folding in of the longitudinal edges of the strip prior to the winding thereof, the double thickness of the strip at the ends of the roll thus providing hard or solid ends for the roll and leaving the intermediate adhesively coated portion of the roll soft and free of pressure. Moreover, the wax coating applied to the back of the strip will prevent sticking of the composition treated side of the strip to the back thereof when wound into a roll as well as enhance the moisture proof and vapor proof properties of the finished sheets.

In applying strips or sheets provided by the present invention to heat insulating material such as used in building construction, the strip A having the adhesive composition thereon may be conveniently applied, for example, to a strip 31 of rock wool, glass wool or other insulating material suitably fed from a storage bin 32 as shown in Fig. 9, the strip A of paper or the like having the adhesive composition thereon being supplied from the roll A' and fed around a roll 34 so that the ribbed composition treated side of the strip is applied against the insulating material, the roll 34 being suitably heated so that heat is applied to the strip at a sufficiently high temperature, as within the range hereinbefore stated, to soften the composition and render it viscous. The heated adhesive strip and the strip 31 of rock wool or the like are then pressed together, as by passing them between a series of press rolls 35, and the strips A and 31 are then cooled to ordinary temperature, as by passing them through a chamber 36 which may be air cooled, and the strips may be finally cut off into batts of the desired length, as shown for example in Fig. 10. Upon cooling to ordinary atmospheric temperature, the composition on the sheet A<sup>2</sup> will adhesively secure the batt 31<sup>a</sup> thereto.

The edges such as a<sup>2</sup> and a<sup>3</sup> of the sheet A<sup>2</sup>, which are uncoated with the composition, preferably project beyond the edges of the batt 31<sup>a</sup> and are left free so that when the batt is placed in position in a wall, as shown in Fig. 11, these edges of the sheet may be extended and nailed or otherwise secured to the studding 37, thus holding the insulating material in place in a wall. When used in this way, the composition on the sheet serves not only to secure it to the insulating material but it also provides a moistureproof backing for the insulating material which will protect it against saturation with moisture from fresh plaster applied to the wall, and the sheet will assist the insulating material in insulating

the wall by preventing circulation of air through the wall.

It has been found that by providing the sheet with the adhesive composition the surface of which is ribbed, a more effective bond is obtained between the sheet and the insulating material, especially when fibrous or filamentary material such as rock wool or glass wool is applied thereto, than is obtainable with an adhesive having a flat surface, since the fibres or filaments of such insulating material will settle into the softened ribs when applied thereto.

We claim as our invention:

1. The process of producing a sheet of flexible water-proof material possessing adhesive properties when heated, which comprises applying to the entire surface of a strip of cellulosic material a coating of a normally solid heat sensitive mixture of substantially equal proportions of montan pitch and an adhesive substance selected from the group consisting of an asphalt and stearine pitch while heated to a temperature sufficient to liquefy it, forming the coating thus applied to the strip, while sufficiently cooled to become plastic, into ribs, and then cooling the coating to harden it.

2. The process of producing a sheet of flexible water-proof material possessing adhesive properties when heated, which comprises applying to the entire surface of a strip of cellulosic material a coating of a normally solid heat sensitive mixture of substantially equal proportions of montan pitch and an adhesive substance selected from the group consisting of an asphalt and stearine pitch while heated to a temperature sufficient to liquefy it, cooling the coating sufficiently to render it plastic, forming the coating thus applied to the strip into ribs and simultaneously removing the coating from marginal edges of the strip while the coating is plastic, and then cooling the coating to harden it.

3. The process of producing a sheet of flexible material possessing adhesive properties when heated, which comprises applying to the surface of a strip of material a coating of a normally solid heat sensitive mixture while heated to a temperature sufficient to liquefy it, said mixture being adhesive when heated but substantially non-tacky at ordinary atmospheric temperature, removing the coating, while cooled sufficiently to become plastic, from marginal edges of the strip, folding said edges of the strip inwardly, and then forming the strip into a roll.

4. The process of producing a sheet of flexible material possessing adhesive properties when heated, which comprises applying to the entire surface of a strip of material a coating of a normally solid heat sensitive mixture while heated to a temperature sufficient to liquefy it, said mixture being adhesive when heated but substantially non-tacky at ordinary temperature, forming the applied coating into ribs and simultaneously removing the coating from marginal portions of the strip while said coating is cooled sufficiently to become plastic, cooling the coating sufficiently to harden it, folding the marginal edges of the strip inwardly, and forming the strip into a roll.

5. The process of producing a sheet of flexible material possessing adhesive properties when heated, which comprises applying to the entire surface of a strip of material a coating of a normally solid heat sensitive mixture while heated sufficiently to liquefy it, said mixture being adhesive when heated but substantially non-tacky

at ordinary temperature, forming the applied coating into ribs and simultaneously removing the coating from marginal portions of the strip while said coating is cooled sufficiently to become plastic, applying a coating of wax to the opposite surface of the strip, cooling the strip sufficiently to harden both of said coatings, folding the marginal edges of the strip inwardly, and forming the strip into a roll.

6. A sheet of flexible waterproof material possessing adhesive properties when heated, comprising a sheet of cellulosic material having applied to a surface thereof a ribbed coating of a normally solid heat sensitive mixture of substantially equal proportions of montan pitch and a

substance selected from the group consisting of an asphalt and stearine pitch which is substantially non-tacky at ordinary atmospheric temperatures but is adhesive above such temperatures.

7. A sheet of flexible waterproof material possessing adhesive properties when heated, comprising a sheet of cellulosic material having ribs of a normally solid heat sensitive mixture of montan pitch and a substance selected from the group consisting of an asphalt and stearine pitch applied to a surface thereof in an area spaced inwardly from edges thereof.

DONALD B. WHEELER.  
JAMES D. GRIFFIN.